

## UNITED STATES PATENT OFFICE

2,267,758

## INK FOR TEXTILE MARKING

Francis M. Sell, Cincinnati, Ohio, assignor to The National Marking Machine Company, Cincinnati, Ohio, a corporation of Ohio

No Drawing. Application May 20, 1937,  
Serial No. 143,853

21 Claims. (Cl. 250—71)

The object of my invention is to provide an ink for textile marking, by the use of which the marked textiles may be subjected to ordinary laundering or cleaning operations or the like, and thereafter the marks will be (when exposed to ordinary lighting) substantially invisible on all colors and types of textiles and may be rendered clearly visible upon the application of rays of suitable wave length or characteristics, particularly a substance which exhibits fluorescence under ultra-violet ray illumination.

This application is in part a continuation of my co-pending application Serial No. 17,334, filed April 19, 1935.

In practice I have demonstrated that my object may be attained by using as the fluorescent ingredient a substantially colorless fluorescent dyestuff, which may be defined as follows: A chemical compound which is substantially colorless (viewed under normal light), highly fluorescent (viewed under ultra-violet rays and in the substantial absence of normal light), and which has the property of being irreversibly transferred from a solution to a textile to which it is applied. The term "colorless fluorescent dyestuff" will be used in that sense hereinafter, in the specification and claims. A "colorless fluorescent dyestuff," may also be defined as a compound which is substantive to textile fibers and which on the fibers is substantially invisible under normal light but fluorescent under filtered ultra-violet rays. More technically I may describe this compound as having either no chromophoric groups, or weak chromophoric groups, strong fluorophoric groups and strong auxochromic groups.

To accomplish my object it is essential that this dyestuff remain substantially colorless and fluorescent and that it still adhere to the textile to which it has been applied after that textile has been subjected to an ordinary laundering or cleaning operation or the like.

In the present invention, I employ as the marking ink, a colorless fluorescent dyestuff dissolved in a vehicle. The dyestuff is one that when the ink is printed on the fabric (or otherwise marked thereupon) is colorless when viewed under normal light, but which is strongly fluorescent under ultra-violet rays. It is noted that a dyestuff is a substance which when applied in solution to a textile material, becomes irreversibly attached to said textile material, and the term is so used herein. The dyestuffs used in the present invention are such as do not, when printed on the textile fabric (either before or after laundering or cleaning the fabric) give a color, when viewed under ordinary light, but which do exhibit a strong fluorescence (both before and after laundering or cleaning the fabric) when viewed under ultra-violet rays. The vehicle used in making the ink is one that will be completely or

substantially completely removable from the textile fabric by an ordinary laundering or cleaning operation to which the textile article is subjected.

5 10 One of the dyestuffs which I have used commercially for this purpose has the following structure:



This compound may be classed as stilbene dyestuff. This is substantive to cotton.

Another dyestuff that may be used for this purpose has the following structure:



This compound may be classed as a thiazole dyestuff. This is substantive to both cotton and wool and silk.

20 25 This example is continued from my copending application Ser. No. 17,334 filed April 19, 1935, wherein this particular dyestuff was described as useful for the purpose here employed.

Another dyestuff that may be used for this purpose has the following structure:



This compound may be classed as a coumarine dyestuff. This is substantive to silk and wool.

Another dyestuff that may be used for this purpose has the following structure:



This compound may be classed as a phenylethylene dyestuff. This is substantive to wool and silk.

The general subject of dyestuffs is known to chemists, and the general subject of fluorescence is also known to physicists and to chemists. Obviously, chemists skilled in this art may compound various ingredients which will accomplish the same results as those herein specifically mentioned. Hence, I wish to be understood as not limiting my invention to the specific structure of the dyestuffs mentioned.

It is well known to chemists that certain dyestuffs are substantive to vegetable fibers, such as linen and cotton, and other dyestuffs are substantive to animal fibers, such as silk and wool. There are few dyes, relatively speaking, that are substantive to both vegetable and animal fibers. In order to accomplish my object it is obvious that I may (and preferably do) use two or more of the above mentioned dyestuffs. The reason for this is the fact that laundries usually (or at least frequently) receive, in a parcel of articles to be laundered, several different kinds of articles, made of different kinds of fabrics, e. g. silk or woolen articles and cotton or rayon articles. It is desirable (and from a practical and commercial standpoint essential) that the one stamping ink should be capable of effective use on all the common kinds of fabrics to be encountered, in ordinary goods to be laundered.

In preparing my new ink I dissolve any selected one or more of said dyestuffs in a vehicle which has the following characteristics. Its viscosity is such that when used, for example, with a laundry marking machine it may be transferred from an inking pad to type in the ordinary manner, and then transferred from the type to the textile to be marked in the ordinary manner. It is also necessary that this vehicle must have such a degree of surface tension that when applied to a textile it will not excessively "bleed" and thereby become illegible. Furthermore, it must have a drying rate such that when used, for instance, on a laundry marking machine, it may be transferred from an inking pad to the type and from the type to the textile before undue evaporation. Furthermore, this vehicle must be of such characteristics that when the ink in which the vehicle is used is applied to a textile, the vehicle will permit the colorless, fluorescent dyestuff to "dye" the textile.

By "dye" I mean the irreversible transferring of the dyestuff from the solution to the textile. This is the common usage of the verb "dye."

I have found in practice that the presence of a small amount, at least, of an abnormal liquid, such as water, glycerine, glycols, or the like, causes the vehicle of the ink to act as a dye bath. For certain of my dyestuffs the addition of a weak acid, such as oleic acid, or a weak base, such as triethanolamine, causes the ink to have improved dyeing properties. Such weak acids and bases do not injure the fabric or any colored dye already carried thereon. In this connection I note that many of the articles commonly sent to laundries have been colored (dyed) and with dyestuffs of all the usual types. The vehicle must be without action thereupon, since it is intended not to modify the colors of the articles, in any manner.

Certain of the ingredients that can safely be used in the vehicle of my new inks are: glycerine, ethylene glycol, triethylene glycol, iso propyl alcohol, propyl alcohol, ethylene glycol mono butyl ether, ethylene glycol mono ethyl ether, diethylene glycol mono methyl ether, sulfonated castor oil, oleic acid, triethanolamine, and pine oil.

The vehicle of the ink is thus seen to be composed essentially of materials that are substantially completely removable from the fabric by the ordinary laundering process. Some of the liquid components of the ink are preferably less volatile than water.

I have produced commercially successful ink as follows: 20 gms. of dyestuff, such as the hereinbefore mentioned stilbene dyestuff, are dissolved in 400 ccs. of glycerine, and 100 cc. of iso propyl alcohol and 500 cc. of ethylene glycol mono butyl ether are added and stirred.

Another ink which I have demonstrated as practical is as follows: 20 gms. of dyestuff, such as the hereinbefore mentioned thiazole dyestuff, are dissolved in 500 ccs. of triethylene glycol and 500 ccs. of diethylene glycol mono methyl ether are added.

Another ink which I have demonstrated as practical is as follows: 20 gms. of dyestuff, such as the hereinbefore mentioned coumarine dyestuff, are dissolved in 200 ccs. of glycerine and 200 ccs. of iso propyl alcohol, 100 ccs. of triethanolamine, and 500 ccs. of ethylene glycol mono ethyl ether are added.

Another ink which I have demonstrated as practical is as follows: 20 gms. of dyestuff, such as the hereinbefore mentioned phenylethylene dyestuff, are dissolved in 200 ccs. of glycerine and 200 ccs. of oleic acid, 100 ccs. of iso propyl alcohol and 500 ccs. of ethylene glycol mono butyl ether are added.

The above examples must be considered as representative of a large number of possible types of inks, and I do not wish to be understood as limiting my invention to the specific formulae herein disclosed.

For the purpose of enabling an operator to readily and easily read the identification marks in the textiles after the textiles have been subjected to the laundering or dry cleaning operations, and all normally visible portions of the marks thereby removed, I have commercially successfully accomplished this in the following manner: The textiles are placed in a dimly lighted room and subjected to rays of such wavelength or characteristics that when applied to the mark they will cause the fluorescent ingredient remaining in the textile to become brilliantly fluorescent, to the extent that the mark may be clearly seen at a considerable distance. In practice, I have demonstrated that these rays may be obtained by the use of an ultra violet lamp. I have also found that with filtered ultra violet rays substantially all ingredients having this fluorescent character may be energized to become brilliantly fluorescent. I preferably employ the filtered ultra violet rays because of economy in operation and because they are harmless to the operators. It will of course be obvious that any ultra-violet ray lamp to be used should be one which does not, when in use, give any considerable amount of white light. It is for that reason that I have mentioned filtering the ultra-violet rays, by which means I allow the ultra-violet rays to impinge upon the laundry marks without any considerable amount of light. I use the expression "in the substantial absence of light" in the claims to indicate the absence of more light than would normally be present in a dimly lighted room. I have also demonstrated that so-called X-rays and cathode rays will cause certain fluorescent ingredients under the same conditions to become brilliantly fluorescent, but X-ray and cathode rays will not thus excite as

70  
75

many different kinds of fluorescent compounds as will the ultra violet rays. In view of the foregoing I desire to be understood as including in my invention the use of rays having properties, equivalent for my purpose, to those of ultra violet rays.

In certain of the appended claims I have included laundering and dry-cleaning, in the generic expression "a cleaning operation," which expression is intended to be substantially equivalent to a laundering or dry-cleaning operation.

My new ink as covered in the present application, is now being commercially used in numerous laundries throughout the United States and principal foreign countries, and it is the general practice to use it as follows: When used on a laundry marking machine a small quantity of the ink is poured upon the inking pad. Then the textile to be marked is placed upon the platen and the marking machine operated to press the type first upon the pad and then upon the textile. When this has been done a large portion of the ink is deposited upon the surface of the article, but a sufficient quantity is pressed into or absorbed by the fibers so that after the textile is subjected to a laundering or cleaning operation and the surface ink all or partly removed, there will remain enough of the fluorescent ingredient to define the mark thus printed. After the laundering or cleaning operation the textile is subjected to the action of the ultra violet rays and the mark caused to become brilliantly fluorescent and clearly visible to the operator. Heretofore, with the use of indelible colored ink for laundry marking purposes it was the custom to employ type of smallest possible size and to place the mark in concealed, relatively inaccessible portions of the textile. This was for the purpose of making the laundry marks inconspicuous on the laundered articles. With my improved ink it is now the common practice to employ type of relatively large size and to place the mark in conspicuous and readily accessible portions of the textiles, for instance upon the outer upper surface of folded handkerchiefs. Hence, in assorting the articles into customers' bundles much time is saved and so-called "shorts and longs" in a laundry are substantially eliminated. Furthermore, much of an operator's time is saved in the marking operation because the operator does not need to hunt for a concealed or inaccessible portion of the textile.

Laundries and dry cleaning establishments which are now using my new ink have entirely eliminated the great objection to their work caused by the presence of black identification marks on all laundry articles, and in addition have effected a substantial economy in the operation of the marking and redistributing departments.

I claim as my invention:

1. An ink for textile identification marking which comprises a vehicle and a plurality of substantially colorless fluorescent organic dyestuffs dissolved therein, said dyestuffs being invisible on any fabric to which they are applied, when viewed under ordinary light, but visible on said fabric when viewed under ultra-violet rays in the substantial absence of light, and said dyestuffs including at least one that is substantive to cellulosic fibres and at least one that is substantive to animal fibres, the vehicle of such ink being sufficiently removable in ordinary cleaning operations to produce substantially no increase in

stiffness in said fabric after such cleaning operation.

2. An ink for textile identification marking which comprises a vehicle and a colorless fluorescent organic dyestuff in solution therein, said vehicle being a viscous liquid and said dyestuff being one that is fast to a cleaning operation and on the textile material is invisible under ordinary light but visible under ultra-violet rays in the substantial absence of light, the vehicle of such ink being sufficiently removable in ordinary cleaning operations to produce substantially no increase in stiffness in said fabric after such cleaning operation.

15 3. An ink for textile identification marking which comprises a colorless fluorescent organic dyestuff carried in a viscous liquid vehicle, which ink is of a consistency suitable for printing identification characters upon fabrics, such dyestuffs 20 being capable of dyeing fabrics when so applied, and when so applied being sufficiently fast to ordinary laundering that the markings are clearly visible under ultra-violet rays in the substantial absence of light, although invisible under ordinary light, after said fabrics have undergone a laundering operation, and said vehicle being substantially entirely removable by an ordinary laundering operation.

4. An ink for textile identification marking, 30 which comprises a colorless fluorescent organic dyestuff capable of exhibiting fluorescence when printed upon a textile material and when exposed to ultra-violet rays, and a vehicle therefor, said ink being of a consistency capable of being 35 printed by type upon a textile material, said dyestuff when so applied to textiles, resisting ordinary laundering operations and resisting dry-cleaning operations, and being thereafter clearly visible and legible when exposed to ultra-violet 40 rays in the substantial absence of light, said vehicle being substantially wholly removable from said textile materials by an ordinary laundering operation and by an ordinary dry-cleaning operation.

45 5. An ink for textile identification marking which comprises a plurality of substantially colorless fluorescent organic dyestuffs and a viscous liquid vehicle therefor, one at least of said dyestuffs being a silk and wool dye and one at least 50 of said dyestuffs being a cotton dye, said dyestuffs being fast to ordinary laundering, and said liquid vehicle being substantially removable by an ordinary laundering, and said ink being of a consistency suitable for being applied to a fabric 55 by means of type, each of said dyestuffs when printed upon a textile product to which said dyestuff is substantive, being substantially invisible under ordinary light but being visibly fluorescent when subjected to ultra-violet rays in a semi-dark room.

60 6. An ink for textile identification marking, comprising a substantially colorless fluorescent organic dyestuff which is fluorescent under ultra-violet rays, dissolved in a vehicle, said vehicle 65 comprising glycerine, iso-propyl alcohol and ethylene glycol mono butyl ether, in the following proportions:

70 Colorless fluorescent dyestuff \_\_\_\_\_ gms. 20  
Glycerine \_\_\_\_\_ ccs. 500  
Iso-propyl alcohol \_\_\_\_\_ ccs. 100  
Ethylene glycol mono butyl ether \_\_\_\_\_ ccs. 500

75 said dyestuff when on a fabric, being fast to an ordinary laundering operation and thereafter being substantially invisible under ordinary light,

but clearly visible under ultra-violet rays, the vehicle of such ink being sufficiently removable in ordinary cleaning operations to produce substantially no increase in stiffness in said fabric after such cleaning operation.

7. An ink for textile identification marking, comprising a substantially colorless fluorescent organic dyestuff and a vehicle therefor comprising glycerine, iso-propyl alcohol and ethylene glycol mono butyl ether, said dyestuff when on a fabric, being fast to an ordinary laundering operation and thereafter being substantially invisible under ordinary light, but clearly visible under ultra-violet rays, the vehicle of such ink being sufficiently removable in ordinary cleaning operations to produce substantially no increase in stiffness in said fabric after such cleaning operation.

8. An ink suitable for textile identification marking which is a viscous liquid vehicle carrying a substantially colorless fluorescent dyestuff having its structural formula selected from the group consisting of



which dyestuff, applied to fabrics is fast to ordinary laundering and leaves on the laundered fabric, a mark which is not visible under ordinary light, but clearly visible under ultra-violet rays in the substantial absence of light, and said liquid vehicle being substantially completely removable by ordinary laundering.

9. An ink suitable for textile identification marking which is a viscous liquid vehicle carrying a substantially colorless fluorescent dyestuff having the structural formula



which dyestuff, applied to fabrics is fast to ordinary laundering and leaves on the laundered fabric a mark which is not visible under ordinary light, but clearly visible under ultra-violet rays in a semi-dark room, and said liquid vehi-

cle being substantially completely removable by ordinary laundering.

10. An ink suitable for textile identification marking which is a viscous liquid vehicle carrying a substantially colorless fluorescent dyestuff having the structural formula



15 which dyestuff, applied to fabrics is fast to ordinary laundering and leaves on the laundered fabric a mark which is not visible under ordinary light, but clearly visible under ultra-violet rays in the substantial absence of light, and said liquid vehicle being substantially completely removable by ordinary laundering.

11. An ink suitable for textile identification marking which is a viscous liquid vehicle carrying a substantially colorless fluorescent dyestuff having the structural formula



which dyestuff, applied to fabrics is fast to ordinary laundering and leaves on the laundered fabric a mark which is not visible under ordinary light, but clearly visible under ultra-violet rays, and said liquid vehicle being substantially completely removable by ordinary laundering.

40 12. An ink suitable for textile identification which comprises a viscous solution, in a liquid vehicle of a substantially colorless fluorescent dyestuff selected from the group consisting of stilbene dyestuffs, thiazole dyestuffs, coumarine dyestuffs and phenylethylene dyestuffs, which dyestuff when applied upon a textile material, is fast to ordinary laundering, and said vehicle being substantially completely removable by ordinary laundering, said dyestuff when printed upon the textile product, being substantially invisible under ordinary light, but being visibly fluorescent when subjected to radiations selected from the group consisting of ultra-violet rays, X-rays and cathode rays, in the substantial absence of light.

45

50

55 13. An ink suitable for textile identification  
which comprises a viscous solution, in a liquid  
vehicle of a substantially colorless fluorescent  
stilbene dyestuff, which dyestuff when applied  
upon a textile fabric article, is fast to ordinary  
laundering, and said vehicle being substantially  
60 completely removable by ordinary laundering,  
said dyestuff when printed upon the textile prod-  
uct, being substantially invisible under ordinary  
light, but being visibly fluorescent when sub-  
65 jected to radiations selected from the group con-  
sisting of ultra-violet rays, X-rays and cathode  
rays, in the substantial absence of light.

70 14. An ink suitable for textile identification which comprises a viscous solution, in a liquid vehicle of a substantially colorless fluorescent thiazole dyestuff, which dyestuff, applied upon a textile fabric, is fast to ordinary laundering, and said vehicle being substantially completely removable by ordinary laundering, said dyestuff when printed upon the textile product, being substantially invisible under ordinary light, but

75

being visibly fluorescent when subjected to radiations selected from the group consisting of ultra-violet rays, X-rays and cathode rays, in the substantial absence of light.

15. An ink suitable for textile identification which comprises a viscous solution, in a liquid vehicle of a substantially colorless fluorescent coumarine dyestuff, which dyestuff, applied upon a textile material, is fast to ordinary laundering, and said vehicle being substantially completely removable by ordinary laundering, said dyestuff when printed upon the textile product, being substantially invisible under ordinary light, but being visibly fluorescent when subjected to radiations selected from the group consisting of ultra-violet rays, X-rays and cathode rays, in the substantial absence of light.

16. An ink suitable for textile identification which comprises a water-soluble viscous liquid solvent that is less volatile than water, containing in solution therein, a substantially colorless fluorescent dyestuff selected from the group consisting of stilbene dyestuffs, thiazole dyestuffs, coumarine dyestuffs and phenylethylene dyestuffs, which dyestuff when applied upon a textile article is fast to ordinary laundering, and said vehicle being substantially completely removable by ordinary laundering, said dyestuff when printed upon the textile product, being substantially invisible under ordinary light, but being visibly fluorescent when subjected to radiations selected from the group consisting of ultra-violet rays, X-rays and cathode rays, in the substantial absence of light.

17. Textile fabric articles of the types commonly subjected to cleaning operations when soiled, carrying identifying marks thereupon, suitable for identifying ownership of the same, such mark consisting of a dyeing with a colorless fluorescent organic dyestuff which, on the textile is fast to an ordinary laundering process and is fast to an ordinary dry-cleaning process, and the said identifying mark being invisible under ordinary light but clearly visible under ultra-violet rays in the substantial absence of light, and the marked area being indistinguishable from the remainder of the fabric except by the said fluorescence which is clearly visible under ultra-violet rays in the substantial absence of light.

18. Textile fabric articles carrying fluorescent identifying marks thereupon, suitable for identifying ownership of the same, such mark consisting of a dyeing with the para-hydroxy compound of dehydro-thio-p-toluidine which, on the textile articles is fast to an ordinary laundering process and is fast to an ordinary dry-cleaning process, and the said identifying mark being invisible under ordinary light but clearly visible under ultra-violet rays in the substantial absence of light, and the marked area being indistinguishable from the remainder of the fabric of said articles except by the said fluorescence which is clearly visible under ultra-violet rays in the substantial absence of light.

19. An article of manufacture comprising a fabric of a character requiring a laundering op-

eration, an identification mark thereon in the form of specific legible characters, which mark is substantially invisible when viewed under ordinary light, and composed of a vehicle of a sticky and viscous substance upon the surface of and penetrated into and around the fibers of the fabric and being of a character substantially wholly removable in a laundering operation, and a colorless organic dyestuff mixed with said vehicle and fixed in the manner of a dye to the fibers of the fabric in the same patterns as that of the vehicle, said dyestuff being one that is fluorescent under ultra-violet rays in the substantial absence of light, but invisible in normal light, and being fast to laundering, when on said fabric.

20. An improvement in the art of fabric article identification marking, which comprises the step of dyeing upon a completely manufactured textile fabric article, an identifying mark comprising characters legible by exposure to ultra-violet rays in the substantial absence of light, and said characters being made with a composition which contains an organic dyestuff carried in a vehicle, said dyestuff being colorless under ordinary light, and the dyestuff when applied on said fabric article being substantially fast to laundering and to dry cleaning operations, and showing fluorescence when subjected to ultra-violet rays in the substantial absence of light, and said vehicle being composed essentially of material which is substantially completely removable from said fabric article during an ordinary cleaning operation, the said marking being left legible on the fabric article by ultra-violet rays in the substantial absence of light, after said cleaning step, whereby on the cleaned article the identification mark is left invisible under ordinary light while remaining visible under ultra-violet rays in the substantial absence of light.

21. An improvement in the art of fabric article identification marking, which comprises the step of dyeing upon a completely manufactured textile fabric article, an identifying mark comprising distinctive characters legible by exposure to ultra-violet rays in the substantial absence of light, said characters being made with a composition which consists essentially of a dyestuff carried in a vehicle, said dyestuff being colorless under ordinary light and including at least one colorless dyestuff selected from the group consisting of a stilbene dyestuff, a thiazole dyestuff, a coumarine dyestuff and a phenylethylene dyestuff, and the dyestuff when so applied on said fabric article being sufficiently fast to laundering and dry cleaning operations and showing fluorescence when subjected to ultra-violet rays in the substantial absence of light, and said vehicle being composed essentially of material which is substantially completely removable from said fabric article during ordinary cleaning operations, the said marking being left legible by ultra-violet rays in the substantial absence of light, on the fabric article after said cleaning step.

FRANCIS M. SELL.